

Nov. 18, 1930.

S. I. CHARLESWORTH ET AL

1,782,341

COATING COMPOUND

Filed Feb. 4, 1927.



Witnesses:

Edwin Truel

Inventors:

STANTON I. CHARLESWORTH and  
ARCH W. HARRIS.

By *D Anthony Duna*

Their Attorney.

## UNITED STATES PATENT OFFICE

STANTON I. CHARLESWORTH AND ARCH W. HARRIS, OF CLEVELAND, OHIO

## COATING COMPOUND

Application filed February 4, 1927. Serial No. 165,870.

This invention relates to coating compounds and more particularly to coating compounds suitable for coating nails and other metal objects.

5 One object of this invention is to provide a valuable and commercial coating compound, the principal ingredient of which is recovered from the heretofore waste product known as pure still residue, remaining after 10 the distillation of the light oils recovered from by-product coke oven gas.

Another object is to provide a novel method of manufacturing coating compounds from the heretofore waste pure still residue.

15 In the drawings we have shown a plan of the apparatus used in carrying out our invention.

In the manufacture of by-product coke or other destructive distillation of coal the gases 20 and products of combustion are collected in suitable mains or conduits so that they may be passed through successive processes to recover the by-products therefrom. The specific steps of the various processes differ 25 slightly, but are well-known to those skilled in the art.

The gases after leaving the ovens are first treated to extract the ammonia and tar contents therefrom. The gases are then scrubbed 30 with suitable wash oils to absorb the light oils which are a combination of benzol, toluol, and xylenes.

The wash oils with their content of absorbed light oils (known as benzolized wash 35 oil) are then run through the primary stills to separate the light oils from the wash oils, after which the wash oils are returned to again be used in scrubbing other gases. The separated light oils are then again distilled 40 in what is known as a crude still to separate the light oils from any residue of the wash oils.

During the distillation in the crude still the light oils may be fractionated or may be 45 run over in combination, as desired. However, in either case, the light oils after passing from the crude stills are washed with sulfuric acid to remove impurities such as phenines, phenols, and sulfur compounds.

50 After the light oils are washed with the

sulfuric acid, they have their acid content neutralized with caustic soda or the like, forming a sludge, which sludge will be drained off leaving pure washed light oils, which oils are then distilled in what is known as the pure stills where the light oils are distilled, the distillates being fractionated so as to provide commercially pure benzol, toluol, and xylenes.

55 The residue remaining in the pure stills after distilling the light oils consists of a resinous product composed of resinous polymers resulting from the washing of the light oils with the sulfuric acid, together with some oil. This residue has been heretofore 60 considered a waste product.

65 In accordance with this invention, the residue from the pure stills is collected and charged into a still equipped to distill under a vacuum. The still is then heated to a temperature up to 225 to 300 degrees centigrade under a vacuum of approximately 28 inches of mercury, until the residue has a melting point of 105 to 110 degrees centigrade, and the distillate, which is an intermediate product of polymerization, is permitted to run 70 over from the still into a condenser and collected, forming a commercially usable and salable oil. The residue remaining in the still is a resinous product which is run into a cooling tank and mixed, while molten and hot, with a solvent such as benzol or other light oil products, and made fluid so as to be 75 usable as a coating compound.

80 Referring particularly to the drawings, the letter A designates a tank car or other container constituting the source of supply of the pure still residue which has been formed as set forth in the forepart of this specification. The pure still residue is pumped through a conduit or pipe 2 and discharged into a still 85 3, which may be of any well-known design, but is preferably of the indirectly heated type and sufficiently tight to permit the forming of a vacuum therein. A vacuum pump 4 is connected to a vacuum tank 5 by a pipe 6, which in turn is connected with a condenser 9 by a pipe 7, and the condenser 9 is connected to the top of the still 3 by a pipe 10 so as 90 to receive the distillate from the still, which 95 100

distillate is condensed and collected in the condenser and is a finished oil product. The distillate is an oil consisting of the intermediate product of polymerization and has a low solidifying point so as to be usable in very low temperatures, and also this oil has a base gravity approximately equal to water so as to be ideally usable for lubricating purposes, as a substitute for water in gages, and for the carbureting of water gas.

The still 3 is preferably heated to such a temperature as will give the proper melting point to the residue, but not materially above such point since too high a heat will destroy the resinous residue remaining after the distillation of the above oil. The vacuum pump 4 serves to produce a vacuum of approximately 28 inches of mercury in the still 3 and, therefore, permits the use of the low distilling temperature stated above.

The resinous residue remaining in the still 3 after the distilling off of the oil is then run, while hot, from the still 3 through a pipe 12 into a cooling and mixing tank 13. The tank 13 is provided with a mixing paddle 14 for mixing the residue with a quick drying solvent such as motor benzol, which enters the tank 13 through a pipe 15 from a supply tank 16. A reflux condenser 17 is connected to the tank 13 for condensing and collecting the fumes and vapors from the mixing tank 13.

The resinous residue from the still 3 is sufficiently fluid while hot and molten to readily mix with and be dissolved by motor benzol or a similar solvent, and when so mixed and dissolved forms a very valuable product in the form of a coating material especially adapted for coating nails and the like.

The residue from the still 3 is preferably mixed with about 30 per cent. by weight of motor benzol or other light oil products under the reflux condenser 17, which benzol is added gradually from the supply tank 16 and the mass is stirred continuously so as not to lose any of it through the reflux condenser. The finished material should have a viscosity of approximately 78 degrees as determined by a Doolittle viscosimeter at 104 degrees Fahrenheit, and may then be thinned down by the addition of benzol to any desired viscosity.

Material made as described, forms a varnish-like coating that, while especially adapted for coating nails so as to resist any pulling action which would tend to withdraw the nails from the wood into which they have been driven, may also be used for coating other materials.

While we have described certain specific steps of our method for producing this novel coating material, it will be understood that we do not wish to be limited thereto since various changes in proportions, temperatures and sequence of steps may be made without

departing from the scope of our invention as defined in the appended claims.

We claim—

1. A coating compound adapted to form a hard resinous coating on metal or other surfaces, comprising a resin base consisting of the residue remaining after the distilling, up to 300 degrees centigrade under approximately 28 inches of vacuum, of the pure still residue remaining after the distillation of the light oils recovered from by-product coke oven gas, said resin base being mixed while molten and hot with approximately 30 per cent. by weight of benzol or other light oil products.

2. The method of making a coating compound, which consists in distilling a resinous compound composed of resinous polymers and oils remaining after the distillation of the light oils recovered from by-product coke oven gas at a temperature of from 225 to 300 degrees centigrade and under a vacuum of approximately 28 inches of mercury, until the residue has a melting point of 105 to 110 degrees centigrade, separating the distillate from said compound, then mixing the molten and hot residue with approximately 30 per cent. by weight of benzol to form a fluid coating material having a resinous base.

In testimony whereof, we have hereunto signed our names.

STANTON I. CHARLESWORTH.  
ARCH W. HARRIS.

100

105

110

115

120

125

130